

## UNITED STATES PATENT OFFICE

GEORGE A. RICHTER AND MILTON O. SCHUR, OF BERLIN, NEW HAMPSHIRE, ASSIGNEES  
TO BROWN COMPANY, OF BERLIN, NEW HAMPSHIRE, A CORPORATION OF MAINE

## PROCESS OF REFINING CELLULOSE PULP

No Drawing.

Application filed May 27, 1934. Serial No. 716,154.

This invention has for its object the treatment of cellulose pulp produced by a digestion of raw cellulosic material, and more especially sulphite pulp, to produce a refined pulp having a high color and a great proportion of resistant or alpha cellulose and to accomplish this result with a high yield and with a small proportion of reagents.

Raw sulphite pulp is characterized by a relatively low pentosan content as compared with that of a pulp initially produced by an alkaline digestion, but it contains relatively larger proportions of less-resistant celluloses, such as beta and gamma celluloses, which are largely removed in the soda or sulphate process.

The present invention, in addition to the objects first mentioned, has also for its objects to produce a product which is low in pentosan content and, while low in potash solubility, nevertheless has a high percentage of alpha cellulose, so that it is available not only for the production of cellulose esters, e. g., nitrocellulose or cellulose xanthate, but also for the production of a paper which has a marked similarity to paper produced from cotton rags, in its strength, softness, folding endurance, and resistance to tear.

In carrying out our process three operations are performed, the first of which is a treatment of the pulp with a relatively small proportion of an oxidizing agent for the purpose of removing or dissolving some of the resinous or ligneous components of the pulp and of rendering some of the more refractory components more readily soluble in the alkaline treatment to be described. This treatment is in no sense a bleaching operation, as it does not have the effect of whitening the pulp. The oxidizing reagent reacts with the resins and the more susceptible ligneous content of the pulp, and by the elimination thereof increases the proportion of the resistant or alpha cellulose in the total pulp. Any suitable oxidizing agent may be employed for this purpose, such as calcium hypochlorite or chlorine, but care should be taken to employ only a small proportion of the reagent such as will not react appreciably with the cellulose fibers. After this operation is per-

formed, the resulting product is preferably washed to free it from the reaction products. The second step of our process consists in subjecting the pulp to an alkaline liquor with the application of heat until the alkali has dissolved the greater portion of the non-resistant (beta or gamma) cellulose, and has dissolved the residual reaction products resulting from the first reaction as well as other resinous or ligneous matter which may remain in the pulp. As a result of this operation, the proportion of resistant cellulose to the total quantity of pulp is materially increased. The pulp is now washed thoroughly to remove all of the alkali and the reaction products, and is then subjected to the third operation which consists in bleaching the pulp with calcium hypochlorite or other suitable bleaching agent. The effect of this operation is to remove such coloring matter as may remain in the pulp without materially affecting the proportion of resistant pulp to the total pulp content. After this operation has been concluded, the pulp is now washed again thoroughly and treated with antichlor.

We have found that, by following a process such as herein described, it is possible to effect marked economies in the cost of the reagents employed and at the same time to secure a high yield based on the initial unbleached pulp, and to produce a pulp having a maximum proportion of resistant cellulose. As illustrating more in detail how the process may be carried on in connection with sulphite pulp produced from spruce, the characteristics of which depend more or less upon the varying factors of the fiber-liberating process by which it is produced, it may be assumed, for example, that the unbleached pulp has a total cellulose content of, say, 96.8%, about 85% resistant or alpha cellulose, with a copper number of approximately 3.5. A 10% stock suspension of this pulp is now placed in an open vat, and there is added thereto from 1% to 2% of bleach powder in solution based on the weight of the fiber and on calcium hypochlorite powder containing 35% available chlorine. In lieu thereof we may employ from 0.3% to 0.6% chlorine based on the pulp. The mass is subjected

to agitation for about thirty minutes. As previously stated, the oxidizing agent reacts with the more susceptible ligneous content of the pulp without affecting any material or perceptible bleaching operation upon the pulp. In fact, the pulp appears to be of a darker color when subjected to this treatment than before. As a result of this step of the process, experience has shown that 5 the product after washing contains about 97.2% total cellulose, about 87% to 88% resistant or alpha cellulose, and that the copper number is reduced to about 3. The pulp is now transferred to an open vat and there is 10 added thereto an alkaline liquor of a strength of 0.1% to 0.5% caustic soda or from 1% to 5% caustic soda based on dry pulp. For this purpose we may use as the alkaline reagent either caustic soda or caustic potash 15 or a sodium carbonate or other alkaline solution. The pulp is digested preferably at atmospheric pressure but with the application of sufficient heat to effect the reaction of the mass in from, say, two to six hours. 20 During this operation the free alkali dissolves the greater portion of the non-resistant cellulose—beta and gamma cellulose—as well as the residual undissolved reaction products resulting from the first reaction, and such 25 other resinous or ligneous matter as was not affected by the treatment with the first oxidizing agent. At the end of the period of digestion, the pulp is now thoroughly washed for the removal of all of the reaction products, and experience has shown that at this 30 stage the mass contains about 99.3% total cellulose, about 93% to 94% resistant cellulose, and has a copper number of about 2. The material is now ready for the bleaching 35 action, by which practically all of the coloring matter is removed and the pulp is bleached to the desired degree of whiteness. In this case the pulp is subjected to the bleaching action of the equivalent of from 2% to 40 4% of 35% bleach based on the pulp—calcium hypochlorite being preferably employed for this purpose. As a practical matter, the stock may be in the form of a 10% suspension and the operation may be carried on at a 45 temperature of about 80° F. for from, say, six to eight hours. The pulp is then thoroughly washed and treated with calcium bisulphite, or other suitable antichlor, to neutralize any bleach that may remain in the 50 product. At this point we have found that the stock contains about 99.6% total cellulose, about 92% to 93% resistant or alpha cellulose, and that the stock exhibits a copper 55 number of about 2.3. Instead of carrying on the third step with hypochlorite alone, we may combine with the hypochlorite a certain proportion of caustic soda or sodium carbonate, which has the effect of preventing 60 localized overbleaching and retards the 65

bleaching operation, as pointed out in our application Serial No. 716,153 filed concurrently herewith, and issued as Patent No. 1,639,704, on August 23, 1927. If the reagent for the bleaching operation consists 70 of a mixture of calcium hypochlorite and caustic soda, the final product will contain approximately 99.6% total cellulose, 93% to 94% alpha cellulose, with a copper number of about 1.7. In carrying on the process 75 herein described, there is a much smaller consumption of bleach with a higher pulp yield having a higher percent. of resistant cellulose than has heretofore been possible with the ordinary bleaching operations. In 80 fact, although the total cellulose yield based on the initial unbleached pulp is somewhat lower (from 10% to 15%) than with the usual bleaching operation, there is only about one-half of the amount of bleach used in 85 carrying out our process than is employed in the usual bleaching operation. There is produced as a result of our process, however, a cellulose product which lends itself for the 90 production of cellulose nitrate and other cellulose esters. The average fiber length of the stock is nearly double that of stock produced by the ordinary bleaching methods. A paper produced from the pulp is much softer and at 95 the same time possesses a greater tearing resistance than the paper made from ordinary bleached pulp. It will be seen that cellulose pulp such as we have herein described as resulting from the practice of our process is 100 comparable in value with cotton in the production of cellulose esters, cotton having ordinarily a copper number of, say, 1.5 and comprising, say, from 94% to 96% alpha cellulose, but has a great advantage over cotton 105 in point of economy.

While in the example we have given as illustrating how the process may be practised we have indicated certain values which we have obtained and have also stated specific proportions of the several reagents, we would 110 not consider it a departure from the scope of this invention if these proportions were somewhat changed, assuming that comparable results are secured. In carrying on experimental work in connection with this process, we have noted that when unbleached chemical wood pulp is subjected to the action of an oxidizing agent, with a given proportion of the reagent during a given period of time, 115 the first consumption of the oxidizing agent is accompanied by a rise in the proportion of alpha cellulose in the pulp, but that a critical point is reached so that the further consumption of the oxidizing agent is accompanied by a marked decrease in the proportion of the alpha or resistant cellulose content of the pulp. We have also noted that the copper number decreases with the first consumption of the oxidizing agent up to the 120 125 130

critical point and thereafter rises. Consequently, in carrying on the first step of our process, we employ a relatively small amount of oxidizing agent,—that is, based on the 5 amount of pulp,—and terminate the operation when or before this critical point is reached, this taking about thirty minutes under the conditions stated in the specific example. In the second step of the process, 10 however, the reaction with the alkaline liquor is carried on until the less resistant cellulose is dissolved and removed without effecting a marked deterioration in the alpha cellulose. This may be favored by adding the total quantity 15 of alkali from time to time in relatively small proportion so as to prevent an over-concentration. In the bleaching operation, however, it may be stated that this is carried on until the desired color has been achieved 20 by the dissolving and removal of the coloring matter, and here again care should be exercised to prevent any local overbleaching.

While for the purpose of producing a white product having desirable papermaking and 25 esterification characteristics it is desirable to follow sequentially the three major steps which we have herein described, nevertheless where the whiteness of the final product is not essential in the manufacture of a paper 30 such as ordinarily made from colored rags, we may omit the first and/or third steps, and subject the sulphite pulp to only a digestion with alkali under atmospheric pressure. It may be pointed out, in this regard, that in digesting 35 the pulp at atmospheric pressure with heat, we secure certain advantageous results and marked economy of operation. That is to say, this makes possible a continuous operation in open vessels, thus ensuring simplicity of operation and ease of control. Again, we 40 secure an economy in the use of steam in heating, and maintain the heat of the alkaline stock suspension; a greater yield of product based on original raw sulphite pulp is secured 45 than where the pressure digestion is employed; and, owing to the fact that in digesting under atmospheric pressure the temperature to which the mass is heated is consequently limited, we prevent the degradation 50 of the alpha cellulose content and yet secure the selective reaction of the less-resistant celluloses and thereby produce a product which when made into paper has a greater strength, resistance to tear, and folding endurance than 55 one which has been digested under pressure.

What we claim is:

1. A process which comprises treating unbleached, previously-liberated pulp with an oxidizing agent until the residue from this 60 treatment shows a maximum alpha cellulose content, and then treating this high alpha-cellulose-containing residue with an alkaline liquor under conditions to increase further the alpha cellulose content of the residual pulp, 65 thus preserving or developing in the fibres

the most desirable paper-making characteristics.

2. A process which comprises treating unbleached wood pulp with an oxidizing agent until the residue from this treatment shows a maximum alpha cellulose content, and then digesting this high alpha-cellulose-containing residue in an alkaline liquor under conditions to increase further the alpha cellulose content of the residual pulp, thus preserving 70 or developing in the fibres the most desirable paper-making characteristics, and bleaching the digested pulp.

3. A process which comprises treating unbleached chemical pulp with an oxidizing agent until the residue from this treatment shows a maximum alpha cellulose content, washing the residue, digesting the washed residue in an alkaline liquor under atmospheric pressure under conditions to increase further the alpha cellulose content of the residual pulp, thus preserving or developing in the fibres the most desirable paper-making characteristics, again washing the digested pulp, and bleaching the washed pulp in a hypochlorite bleach liquor containing sufficient free alkali to maintain a condition of distinct alkalinity throughout the bleaching operation.

In testimony whereof we have affixed our signatures.

GEORGE A. RICHTER.  
MILTON O. SCHUR.

100

105

110

115

120

125

130